# EUROPEAN PATENT SPECIFICATION

(11) **EP 0 588 461 B1**
(45) Date of publication and mention of the grant of the patent: **14.05.1997**
(21) Application number: 93301815.2
(22) Date of filing: 10.03.1993
(51) Int. Cl.: H01B 12/00, H01R 4/68

(54) **Superconductive current lead**
Supraleitende Stromzuführung
Amenée de courant supra-conductrice

(30) Priority: 14.09.1992 JP 244966/92
(43) Date of publication of application: 23.03.1994
(73) Proprietor: HITACHI CABLE, LTD., Chiyoda-ku Tokyo 100 (JP)
(72) Inventor: Sasaoka, Takaaki, Tusuchiura-shi, Ibaraki-ken (JP)
(74) Representative: Jackson, Peter Arthur

(56) References cited:
- EP-A- 0 409 150
- EP-A- 0 428 993
- JP-A- 3 276 521
- JP-A- 4 155 715
- US-A- 5 075 285

## Description

This invention relates to a superconductive current lead, and more particularly to a superconductive current lead for connecting a superconductive machine placed in an atmosphere at an extreme low temperature to a power supply, etc. placed in an atmosphere at room temperature.

A current lead which is used for a superconductive machine is designed to have a cross-section, such that the sum of heat generated by the current flow through the current lead and heat transferred from a high temperature portion to the current lead becomes minimum, and an evaporation amount of coolant such as helium, etc. becomes also minimum.

In conventional cases, a current lead is composed of copper wires. Under this circumstance, a current lead using oxide system superconductive wires each covered with an Ag layer has been studied for the same purpose.

A current lead composed of an Ag-layered oxide system superconductive wires, however, has the disadvantage in that the amount of heat transferred is large, because the thermal conductivity of Ag is large, at an extreme low temperature region, which is an operating region of a superconductive machine, as compared to other metals, although this results in an advantage in that the stability of the superconductive wires is increased.

In this current lead, there is a further disadvantage in that Joule heat generated by eddy currents and coupling currents of the Ag layers is not negligible, because the electric resistance of the Ag layers becomes very small at an extreme low temperature, when AC current or transient current flows through the current lead.

JP-A-4155715 and US-A-5975285 disclose a superconductive current lead comprising one or more superconductive wires, the or each wire including a first member of an oxide system superconductive material and a second member of an Ag-Au alloy. According to the present invention, such a lead is characterised in that the alloy is an Ag-Au alloy including Au of less than 15 atomic %, the alloy having a thermal conductivity at a temperature lower than room temperature which is lower than its thermal conductivity at room temperature.

In the alloy used, lowering the thermal conductivity is associated with raising the electric resistance, so that a decrease in eddy current loss or coupling current loss is realized, when AC current or transient current flows through the superconductive current lead.

In the invention, an oxide system superconductive material may be a material selected from, for instance, Y-Ba-Cu-O, Bi-Sr-Cu-O, Bi-Pb-Sr-Ca-Cu-O, Tl-Ba-Cu-O, Tl-Ba-Ca-Cu-O, Tl-Sr-Ca-Cu-O, La-Sr-Cu-O, La-Ba-Cu-O.

A barrier layer of precious metal may be interposed between the oxide system superconductive material and the lower thermal conductivity alloy.

The content of Au in the alloy is preferably 1 to 10%, by atomic ratio.

A predetermined number of superconductive wires may be one or more superconductive wires.

In the accompanying drawings:
Fig.1 is an explanatory diagram showing a superconductive current lead connecting a superconductive machine to a power supply ;
Fig.2 is a perspective view showing a superconductive current lead of a first preferred embodiment according to the invention ; and
Fig.3 is a perspective view showing a superconductive current lead of a second preferred embodiment according to the invention.

Fig. 1 shows a superconductive current lead 4 connected to a superconductive coil (machine) 3 and a current lead 5 by connectors 41 and 42, and a power supply 6 provided to apply a predetermined voltage across the superconductive coil 3 via the current lead 5 and the superconductive current lead 4, wherein the superconductive coil and current lead 3 and 4 are immersed in liquid helium 2 contained in a container 1.

Fig.2 shows a superconductive current lead 4 of a preferred embodiment according to the invention which is used in the apparatus as shown in Fig.1. The superconductive current lead 4 comprises a plurality of tape-shaped wires 7 each comprising a core 8 of an oxide system superconductive material and an alloy covering layer 9.

In an example of the first preferred embodiment, the core 8 is of an oxide system superconductive material (Bi-Sr-Ca-Cu-O) Bi-2212 system as a main component, and the alloy covering layer 9 is of Ag-3 atomic % Au alloy, wherein each superconducting tape is 2.4 mm in width, 1.4 mm in thickness, and 3.3 mm² in cross-sectional area.

A critical current of this superconductive current lead 4 immersed in the liquid helium 2 at a temperature of 4.2K is 10⁵ A/cm² which is the same value as a value obtained in case where pure Ag is used for a covering material. At the same time, a resistivity which is as high as 0.7 to 1.2 µ Ω ·cm is obtained to represent a significant change as compared to the case where pure Ag is used at an extreme low temperature region for a covering material.

In relation to the resistivity of the alloy covering layer 9, a thermal conductivity of the superconductive current lead 4 is smaller than that of common current lead of phosphorus-deoxidized copper. Consequently, the superconductive current lead 4 can be used with an eddy current loss of one percent as compared to that in the case where pure Ag is used for a covering layer.

In regard to electric resistance of the connectors 42 and 41, the resistance value is not only decreased, but also stabilized upon the elapse of time.

The thermal conductivity (W/m · k) of the alloy covering layer 9 is shown below in a table relative to a temperature along with that of a pure Ag covering layer.

| TEMPERATURE (K) | EXAMPLE | PURE Ag |
|---|---|---|
| 260 | 160 | 590 |
| 77 | 51 | 530 |
| 20 | 10 | 25,000 |

Fig. 3 shows a superconductive current lead of a second preferred embodiment according to the invention. The superconductive current lead comprises a basic member 10 of Ag-Au alloy, a thin layer 11 of Ag and an oxide system superconductive layer 12.

As described above, a material representing a lower thermal conductivity at a temperature lower than a room temperature is used for a basic member in the invention, so that a heat transferring through the basic member to coolant is not only decreased, but a heat of the lead generated by the flow of current is also decreased, thereby decreasing the consumption of the coolant and a load of a refrigerator.

A plurality of leads shown in Fig. 3 can be stacked in a similar way to the wires shown in Fig. 2.

## Claims

1. A superconductive current lead comprising one or more superconductive wires (7), the or each wire including a first member (8) of an oxide system superconductive material and a second member of an Ag-Au alloy characterised in that the alloy is an Ag-Au alloy including less than 15 atomic % Au, the alloy having a thermal conductivity at a temperature lower than room temperature which is lower than its thermal conductivity at room temperature.

2. A superconductive current lead according to claim 1, wherein the first member is covered with the second member to provide the superconductive wire; and the predetermined number of superconductive wires are stacked.

3. A superconductive current lead according to claim 1, wherein the first member is layered on one surface of the second member to provide the superconductive wire; and the predetermined number of superconductive wires are stacked.

4. A superconductive current lead according to any one of the preceding claims, wherein the superconductive wire is a tape-shaped wire.

5. A superconductive current lead according to any one of the preceding claims, wherein the alloy includes 1 to 10 atomic % Au.

## Patentansprüche

1. Supraleitende Stromzuführung, mit einem oder mehreren supraleitenden Drähten (7), wobei der oder die Drähte ein erstes Element (8) aus einem supraleitenden Material aus einem Oxidsystem und ein zweites Element aus einer Ag-Au-Legierung enthalten, dadurch gekennzeichnet, daß die Legierung eine Ag-Au-Legierung ist, welche weniger als 15 Atomprozent Au enthält, wobei die Legierung eine thermische Leitfähigkeit bei einer Temperatur geringer als Zimmertemperatur hat, die kleiner ist als ihre thermische Leitfähigkeit bei Zimmertemperatur.

2. Supraleitende Stromzuführung nach Anspruch 1, bei der das erste Element mit dem zweiten Element beschichtet ist, um den supraleitenden Draht zu bilden; und die vorbestimmte Anzahl supraleitender Drähte gestapelt ist.

3. Supraleitende Stromzuführung nach Anspruch 1, bei der das erste Element auf eine Oberfläche des zweiten Elementes aufgeschichtet ist, um den supraleitenden Draht zu bilden, und die vorbestimmte Anzahl supraleitender Drähte gestapelt ist.

4. Supraleitende Stromzuführung nach einem der vorangehenden Ansprüche, bei der der supraleitende Draht ein bandförmiger Draht ist.

5. Supraleitende Stromzuführung nach einem der vorangehenden Ansprüche, bei der die Legierung 1 bis 10 Atomprozent Au enthält.

## Revendications

1. Conducteur de courant supraconducteur comprenant un fil ou plusieurs fils supraconducteurs (7), le fil ou chaque fil comprenant un premier élément (8) d'un matériau supraconducteur du système d'oxyde et un second élément d'un alliage d'Ag-Au caractérisé en ce que l'alliage est un alliage Ag-Au comprenant moins de 15 % d'atomes d'Au, l'alliage ayant une conductivité thermique à une température inférieure à la température ambiante qui est inférieure à sa conductivité thermique à la température ambiante.

2. Conducteur de courant supraconducteur selon la revendication 1, dans lequel le premier élément est couvert avec le second élément pour fournir le fil supraconducteur ; et le nombre prédéterminé de fils supraconducteurs sont empilés.

3. Conducteur de courant supraconducteur selon la revendication 1, dans lequel le premier élément est déposé en couche sur une surface du second élément pour fournir le fil supraconducteur ; et le nombre prédéterminé de fils supraconducteurs sont empilés.

4. Conducteur de courant supraconducteur selon l'une quelconque des revendications précédentes, dans lequel le fil supraconducteur est un fil en forme de bande.

5. Conducteur de courant supraconducteur selon l'une quelconque des revendications précédentes, dans lequel l'alliage comprend 1 à 10 % d'atomes d'Au.
